

# UNITED STATES PATENT OFFICE.

GEORGE H. CAMPBELL, OF TORONTO, ONTARIO, CANADA.

## PROCESS OF PREPARING FLAX.

1,086,270.

Specification of Letters Patent.

Patented Feb. 3, 1914.

No Drawing.

Application filed March 11, 1910. Serial No. 543,699.

To all whom it may concern:

Be it known that I, GEORGE H. CAMPBELL, a citizen of Canada, and a resident of Toronto, in the county of York and Province 5 of Ontario, Canada, have invented certain new and useful Improvements in Processes of Preparing Flax, of which the following is a specification.

This invention relates to the preparation 10 of flax for the various purposes of the textile industry, and has in view a quicker and more economical treatment, and which will produce a greater yield than previously existing processes, all as now will be explained; 15 reference being had to the following specification and claims.

In carrying out this process flax stalks, or straw, in a dry state are passed through a breaking machine which removes the 20 larger portion of the various incrusting matters or shives, the diminution in weight of the straw treated being about 45% of the total original weight.

To render the stalks sufficiently dry, they 25 may be either air dried or dried by the application of heat, the stalks being for this purpose placed on suitable shelves or frames, below which are placed pipes through which passes hot water or steam, heated to a moderate 30 temperature. For most uses and in most instances ordinary air drying will be sufficient, but when the flax stalks are cut before the seeds are matured, to get flax of the highest grade, and if it is desired to break the stalks shortly after cutting, drying by heat will generally be preferable or necessary.

The dried stalks previous to breaking are lightly sprayed or tempered with water 40 alone or water containing in solution a suitable chemical used in very small proportion such as ammonia, sodium carbonate or soap. A small percentage of a suitable oil such as cotton seed oil or paraffin oil may 45 also be held in the alkaline solution in the form of an emulsion. The amount of liquid applied in the operation should be just enough to moisten the fibers which constitute the exterior portion of the stalks, but 50 not enough to sensibly moisten the interior portion or shive material. By this slight preliminary moistening the fibers are rendered more elastic so that they will not break during the operation of breaking, a 55 feature which admits of a very high degree of desiccation previous to the breaking.

The stalks coming from the breaking machines as above described and which still contain a very considerable proportion of the gummy, ligneous and incrusting matter 60 may be used for making rough twine for use as binder twine, grocers' twine and the like.

For use in the various forms of cloth or yarn the product coming from the breaking 65 machine will have to be treated so as to more perfectly eliminate the incrusting or shive constituents. This is done by a process of retting which will now be described, and which may be applied either immediately 70 after the stalks come from the breaking machines or after the fiber has been subjected to the various operations of scutching, hacking, spinning and weaving. In each of those various operations tending to convert 75 the broken stalks into yarn or cloth the material progressively loses a certain amount of the adhering incrusting material or shives but not all, the remaining portion being removed by the process of fermentation retting. 80 There are several methods of fermentation retting that may be used for the purpose, the process of field retting or dew retting being here described in connection with the previous operation of breaking. For 85 this purpose the broken flax straw is spread upon meadows or other forms of open fields and exposed until the residual incrusting matter adhering to the fiber has become sufficiently brittle to be readily removed by subsequent mechanical manipulations such as 90 passing the material through breaking machines, scutching and beating machines or subjecting them to the action of other forms of machines or to manual shive removing 95 operations. The retting may be performed in stages, a portion of the shives being removed after the first exposure and the remainder after the second exposure, which will also have a bleaching effect to a certain 100 extent.

By the breaking of the dry stalks without retting, the greater portion of the shives is eliminated at once whereby the work to be done during the subsequent step of retting 105 is very materially diminished and thus facilitated and shortened. The material on account of the less percentage of incrusting matter contained will also be much lighter than when ordinary field retting without previous breaking is used. The fact that the retting period is shortened has also the

advantage of a very considerable increase in the yield of flax. In the ordinary process of field retting, the yield is only about 10% while by this process it is increased to 15% or even 25%.

After the exposure of the broken flax material for a sufficient length of time to make retting practically complete the flax stalks are passed through a breaking machine preferably with much finer grooves than were used in the original breaking of the dry and unretted flax stalks. If the fiber is retted in the form of yarn, the latter may consist of single strands. If the fiber is converted into cloth before retting this course has the advantage that the incrusting matters are progressively eliminated from the fiber during the operations of twisting the strands and weaving, although the cloth requires more prolonged mechanical treatment after the retting to eliminate all particles of the separated and broken shives. When unretted flax fiber has been converted into cloth or fabric the operation of field retting will be accompanied by bleaching to a greater extent than when more of the shive material is adhering to the fiber, rendering it in fact a simultaneous operation of retting and bleaching.

What I claim as new is:

1. In the art of preparing linen fibers, the improvement which consists in drying, spraying or tempering, and then breaking flax stalks, and retting the resulting material. 30
2. In the art of preparing linen fibers, the improvement which consists in drying, spraying or tempering and then breaking flax stalks, and scutching and retting the resulting material. 35
3. In the art of preparing linen fibers, the improvement which consists in drying, spraying or tempering flax stalks with an aqueous emulsion of an oil, then breaking the stalks, and retting the resulting material. 40
4. In the art of preparing linen fibers, the improvement which consists in drying, spraying or tempering and then breaking flax stalks, converting the resulting material into yarn and retting the latter. 45

Signed at New York in the county of N. Y. and State of N. Y. this 18th day of May A. D. 1909.

GEORGE H. CAMPBELL.

Witnesses:

C. A. O. ROSELL,  
MABELLE A. DAVIS.